

Oct. 29, 1968

S. DAVIES ET AL

3,408,251

TOWS OF SYNTHETIC FILAMENTS AND METHOD FOR MAKING THE SAME

Filed Jan. 11, 1965



1

3,408,251

**TOWS OF SYNTHETIC FILAMENTS AND  
METHOD FOR MAKING THE SAME**

Stanley Davies, 11 Fairfield Estate, Goytre, Pontypool, England; Vincent Leighton Evans, "Yves" Belmont Crescent, Abergavenny, England; and John David Watt, 61 Chequer Road, Doncaster, England

Filed Jan. 11, 1965, Ser. No. 424,563

Claims priority, application Great Britain, Jan. 10, 1964,

1,146/64

6 Claims. (Cl. 161—169)

**ABSTRACT OF THE DISCLOSURE**

A tow and a method for producing said tow which is suitable for stretch-breaking produced by extruding a polyamide having a relative viscosity of less than about 30 into a plurality of filaments which make up the tow. The tow is split into a plurality of bundles or sub-tows and each bundle is then subjected to a different tensioning prior to drawing. The bundles are then reformed into the tow and draw-crimped. The resulting tow has an improved snap-break rating and a more desirable load extension curve.

This invention relates to improvements in or relating to tow and to a method of producing the same, the said tow consisting of filaments of a polyamide, and is particularly concerned with tow which is intended to be converted into slivers and spun into "Schappe-type" yarns.

Tows, such as 100,000 denier 1½ denier per filament 66 nylon tow, intended for the production of "Schappe-type" yarns are converted into slivers on a stretch-breaking machine and the slivers then processed into the spun yarn. A typical stretch-breaking machine is the Seydel-stretch-breaking machine the essential parts of which are briefly described below.

The Seydel stretch-breaking machine consists essentially of two sections, a stretching section and a breaking section. Nearly all of the stretching is done in the stretching section between the various heads of the machine of which there are normally six. Each of these heads consists of a series of rollers in a 3 over 4 arrangement in which there are four positively driven steel rollers with three plastic-covered jockey rollers in the intermediate gaps. The tow is laced through these rollers such that it passes under each of the four steel rollers and over each of the three jockey rollers in succession. The surface speed of the driven rollers in any one head is the same, but the surface speed of the rollers in the different heads increases from the feed (creel) to the delivery end of the machine. The breaking section consists of two pairs of rollers; the near pair, referred to as the intermediate rollers, is at the same time the seventh head of the stretching section since it has a higher surface speed than that of the rollers of the sixth head. The intermediate rollers consist of a positively driven steel roller and a rubber-covered pressure roller, and the front pair of rollers a positively driven steel bottom roller and a leather or rubber-covered top pressing roller. In order that these rollers should be enabled to grip the tow sufficiently tightly to avoid slippage when breaking, the pressure exerted by the rollers is about 400 lb. and 2,500 lb. respectively.

The path of a single tow through the machine is called a channel and the machine may be designed to enable it to take four channels simultaneously.

One of the difficulties encountered in the use of this type of machine is that of so called "snap breaking" which occurs particularly when restarting the machine following a voluntary or involuntary stoppage, although

2

it may also occur during apparently normal running. The snap-break occurs in the stretching section of the machine and results in all of the filaments in one channel of the tow breaking so that the restringing of that tow is necessary. Since the restringing requires that the machine be stopped, there is the possibility that a snap-break will occur in one of the other channels of tow on restart.

It is believed that major factors in the occurrence of snap-breaks in a tow are interfilament adhesion and filament damage caused by the nip of the rollers in the stretching section of the stretch-breaking machine.

Interfilament adhesion increases (a) along the length of the tow in the stretching section and (b) when the tow is stationary in the machine e.g. during a stoppage. The physical factors involved are the tension in the tow due to stretching, the normal pressure of the rollers against the tow and the pressure at the nips between the rollers in each head. The increasing tension in the tow as it travels through the stretching section produces increasing normal and nip pressure as it passes around the rolls. These tensions and pressures are sufficiently great to deform the filaments from circular to hexagonal cross-section and sometimes to cause fusion. These hexagonal filaments will give an increased surface area of interfilament contact and therefore increase the risk of adhesion. Filament adhesion binds the tow either partially or completely into a solid ribbon.

Damage to the filaments between the roller nips introduces a line of weakness across the tow. If one or more of the filaments across this line break soon after restart the relatively unchanged total stress acting on the remaining filaments in the ribbon is excessive and causes more filament breakage. Breakdown of the tow is then rapid and a snap-break frequently occurs.

Filament adhesion is thought to be the most important factor since a snap-break would be initiated by the weaker filaments in the solid ribbon irrespective of the method of weakening these filaments.

It is a necessary feature in the processing of 100,000 denier nylon tows on the stretch-breaking machine as described above, that a large proportion of filaments are broken in the stretching section in order to reduce the strength of the tow sufficiently to prevent slippage at the front pair of rollers in the breaking section. In a tow having high filament adhesion this deliberate breaking action helps to promote snap-breaking at restart and may also be at least partly responsible for these snap-breaks which occasionally occur during normal running.

We have now found that in order to have a good snap-break rating, i.e. a minimal tendency to snap breaking, a tow should have a low breaking load and a wide spread of physical properties, particularly filament extensibility. The low breaking load enables lower tensions being used in the stretching section of the stretch-breaking machine and thus leads to less interfilament adhesion and nip damage, since the lower the tension the lower the pressure at the nip between the rollers. Also a lower tension in the tow means that a smaller percentage of filaments need to be broken in the stretching section to prevent slippage at the front rolls in the breaking section of the stretch-breaking machine. A wide range of filaments extensibilities enables the less extensible filaments to be broken in the stretching section and the strength of the tow reduced before the breaking point for the other filaments has been reached.

The snap-break rating of a tow on a Seydel stretch-breaking machine is determined in the following manner. The overall draft of the stretching section is adjusted so that no tow slippage occurs between the rollers of the breaking section. Four tow channels are used and ten restarts made after voluntary machine stoppages of

5-minutes-duration giving 40 tests per sample. The delivery speed of the tow is set at 96 ft./min. at a breaking section draft of 1.8 and the tests carried out at an ambient temperature of 78° F. and a relative humidity of 60%. The snap-break rating is then calculated from the expression

Percent rating =

$$\frac{(\text{Number of snap-breaks} \times 10) + (\text{Number of very thin places} \times 3) + (\text{Number of thin places} \times 1)}{40 \times 10} \times 100$$

The snap-break rating should be less than 10, and preferably less than 5 if the tow is to be capable of being processed satisfactorily on a stretch-breaking machine.

A "very thin place" exists in a tow when more than 90% but less than 100% of the filaments in the tow break and a "thin place" exists when between 20% and 90% of the filaments break.

Snap break ratings of between 60 and 100 are common for tows which do not have the characteristics of the tows produced by the process of this invention.

Although a tow having a limited spread of physical properties, such as extensibility, can be produced by varying the spinning conditions, a wider and more significant spread can be obtained at the draw crimping stage in the production of tow by using various yarn paths in the squirrel cage of the draw crimping machine.

For the purpose of this description a squirrel cage may be described as an array of bright chrome bars arranged so that the tow can be interlaced through the bars to insert tension in the tow.

Thus by increasing the angle of wrap around the guide bars in the squirrel cage for some of the filaments in the tow and therefore increasing the tension in these filaments relatively to the remainder, the more highly tensioned filaments are stretched or drawn to some extent in the squirrel cage. Because of the stretching of some of the filaments in the tow the draw-crimper draw ratio has to be reduced to prevent breakage of the filaments either in the squirrel cage or in the drawing zone of the draw-crimper. The resulting crimped tow contains filaments drawn to different degrees and hence having a range of filament extensibilities.

A tow having a suitably low breaking load, preferably less than 500 kg./100,000 denier, can be obtained by spinning the filaments constituting the tow from a synthetic high molecular weight polymer, e.g. polyhexamethylene adipamide, having a relative viscosity (R.V.) of 30 or less and preferably in the range 27-30.

Relative viscosity of a polyamide is defined as being the ratio of the viscosity of a solution thereof in ninety percent by weight formic acid containing 11 grams of polyamide per 100 ml. of solution at 25° C., to the viscosity of ninety percent formic acid at the same temperature.

The increase in the range of filament extensibility required in a tow for it to have a good snap break rating can be defined by reference to the load extension curve of the tow. A typical load extension curve for a normal tow consisting of polyhexamethylene adipamide filaments is shown in the drawing curve A in which L is the breaking load in kg., i.e. the maximum load achieved during extension, and S is the length of the "tail" of the load-extension curve. The tail S is defined as being the extension in centimeters required to reduce the load from 200 to 25 kg. In order to have an improved snap-break performance the length of the tail should be at least 1 cm. greater than that of an equivalent tow in which all of the bundles of filaments were subjected to the same tension in the squirrel cage. The effect on the load extension curve of forming a tow from filaments spun from polymer having an R.V. of less than 30 and which have been subjected to different tensions in the squirrel cage is shown by curve B of the drawing. The value of the breaking load, L<sub>1</sub>, is lower and the length of the tail S<sub>1</sub> considerably increased.

The load extension curve is determined using an Instron tensile tester (registered trade mark) fitted with special clamps which are described in British patent application No. 937,818. In the test 20 cm. unsupported length of sample is extended at 50 cm./min.

According to one aspect of this invention therefore, there is provided a process for the production of a tow suitable for stretch-breaking wherein the filaments forming the tow are extruded from a polyamide having a relative viscosity of 30 or less and are subjected to at least two different levels of tension in the squirrel cage of a draw-crimping machine and are then drawn and crimped according to known procedures.

According to another aspect of this invention there is provided a tow consisting of polyamide filaments produced by the above-mentioned process having a snap break-rating (as hereinbefore defined) of less than 10 and having a load extension curve in which the tail (as hereinbefore defined) is at least 1 cm. longer than the tail of the load extension curve of a tow in which all the filaments were subjected to the same tension in the squirrel cage of the draw crimping machine.

The improved stretch-breaking performance of tows produced according to this invention will now be illustrated by the following examples, which examples are in no way intended to limit the scope of the invention.

#### Example 1

A 100,000 denier tow comprising 11 bundles of filaments of polyhexamethylene adipamide (each filament being of 1½ denier) spun from polymer having a relative viscosity (R.V.) of 27 is passed into the squirrel cage of a conventional draw-crimping machine. Five bundles of filaments are passed around the guide bars at a sufficiently high angle of wrap to cause drawing to occur at this stage, the remaining 6 bundles of filaments are passed through at the normal tension. After passing through the squirrel cage the bundles of filaments are recombined and draw-crimped using a draw ratio of 2.64 in the usual manner. The resultant tow had a snap-break rating of 3 when processed on a Seydel stretch breaking machine. The load extension curve for the tow had a tail S of 3.4 cms. An identical tow processed in the same way except that all the bundles of filaments were subjected to the same tension in the squirrel cage and the tow drawn using a draw ratio of 3.0, had a snap-break rating of 98 and the load-extension curve had a tail S of 1.5 cm., i.e. 1.9 cm. shorter than the tow processed according to the invention.

#### Example 2

Two tows identical to those employed in Example 1 were similarly processed but were steam-set for 7 minutes at 25 p.s.i. in a Sanderson steam setting cabinet before testing on the Instron tensile tester. The normal tow had a snap-break rating of 87 and a load extension curve having a tail S of 1.4 cms. whereas the tow containing filaments subjected to different levels of tension had a snap-break rating of 4 and a tail S to the load extension curve of 2.7 cm., i.e. 1.3 cms. longer.

What we claim is:

1. A process for the production of a tow suitable for stretch breaking comprising forming a tow of filaments by extruding said filaments from a polyamide having a relative viscosity of not more than 30, forwarding said tow to the squirrel cage of a draw-crimping machine, subjecting at least one portion of the filaments forming the tow to a different level of tension in said squirrel cage compared to the remainder of the filaments of said tow and then drawing and crimping said tow thereby producing a tow suitable for stretch breaking.

2. A process for the production of a tow suitable for stretch breaking comprising extruding a plurality of filaments from a polyamide having a relative viscosity of not more than 30 to form a tow of said filaments, dividing said tow into at least two bundles of filaments, subjecting

said bundles to different levels of tension prior to drawing and drawing, crimping and recombining said bundles into a tow thereby producing a tow of improved stretch breaking characteristics.

3. A process according to claim 2 wherein the poly- 5 amide has a relative viscosity in the range of 27-30.

4. A process according to claim 3 wherein the poly- amide is polyhexamethylene adipamide.

5. A tow comprising a plurality of crimped polyamide continuous filaments wherein said filaments have a breaking load of less than about 500 kg./100,000 denier and wherein a proportion of said filaments in said tow has a different draw ratio compared to another proportion of filaments in said tow, said tow having a snap-break-rating of less than 10.

6. A tow according to claim 5 wherein the polyamide filaments are polyhexamethylene adipamide filaments.

#### References Cited

##### UNITED STATES PATENTS

2,385,890 10/1945 Spanagel.

3,011,215 12/1961 Alley.

3,114,999 12/1965 Coggeshall.

10 ROBERT F. BURNETT, *Primary Examiner.*

L. M. CARLIN, *Assistant Examiner.*